

## UNITED STATES PATENT OFFICE

2,356,661

## LUBRICATING OIL

Frederick B. Downing, Penns Grove, N. J., and  
Howard M. Fitch, Wilmington, Del., assignors  
to E. I. du Pont de Nemours & Company, Wil-  
mington, Del., a corporation of Delaware

No Drawing. Application April 23, 1942,  
Serial No. 440,200

18 Claims. (Cl. 252—37)

This invention relates to lubricating oils and particularly to lubricating oils designed for heavy-duty service in internal combustion engines.

The production of a satisfactory lubricant, and particularly the production of a suitable lubricating oil for use in internal combustion engines, has presented a very difficult problem and has been the subject of a great deal of research. The problems presented are primarily due to deterioration of the lubricating oil under the conditions of use, which deterioration is primarily the result of oxidation accelerated by heat and the presence of the various metals in contact therewith. The products of such deterioration tend to form sludge, increase the viscosity of the oil, deposit on the parts of the engine and corrode sensitive bearing metals, such as those composed of alloys or mixtures of copper or lead, cadmium and nickel, silver and cadmium, and cadmium and tin. The increase in viscosity, the sludge and the deposits on the parts of the engine impede and may even arrest circulation of the lubricant. Corrosion of the sensitive bearing metals may proceed to such an extent as to cause mechanical failure of the engine. Accordingly, frequent and expensive changes of the oil, reconditioning of the engine and replacement of bearings are necessary. This is particularly true in so called heavy-duty service, that is, in the operation of trucks, buses, stationary and mobile power units and the like, where heavy loads are applied to the engines and deterioration of the oil is accelerated.

Many compounds have been proposed for addition to lubricating oils for the purpose of curing one or more of the defects of the ordinary petroleum lubricating oil. Amongst the materials which have been proposed for addition to lubricating oils are sulfur and sulfur compounds. Sulfur and its compounds are generally added to increase the film strength of the oils. This requires the addition of relatively large proportions of the sulfur and its compounds with sacrifice of other desirable properties of the oil. Usually the sulfur and its compounds tend to increase the corrosion of sensitive bearing metals and to have other deleterious effects, so that they are not ordinarily used, except where high bearing pressures are encountered and it is essential that the oil have a high film strength. Under these circumstances, the disadvantageous properties of the additions are less important and, in some cases, may be overcome by the addition of other materials.

Those skilled in the art have also proposed the addition of soaps and soap-like materials to lu-

bricating oils so as to take advantage of the detergent properties thereof for removing deposits from the parts of the engines and for maintaining the products of deterioration in suspension in the oils. Some of these materials are alleged to inhibit deterioration of the oils, and others are alleged to inhibit corrosion of sensitive bearing metals. Such soaps and soap-like materials are organic compounds containing metals in chemical combination and may generally be referred to as organo-metallic compounds. Generally, the disclosures of the organo-metallic compounds in the art are quite broad and frequently indicate a large number of different metals as being suitable, some of them even indicating that copper compounds would be suitable. Copper and its compounds are notorious as catalysts for the oxidation of organic compounds. Those skilled in the art have generally found that many copper compounds, when employed in lubricating oils in the proportions ordinarily recommended for organo-metallic compounds, actually accelerate oxidation of the oils and/or corrosion of sensitive bearing metals. In the case of those copper compounds which apparently inhibit the formation of sludge and like deterioration products, it has been generally necessary to add relatively large amounts of the copper compound to the oil in order to obtain practical and optimum results. However, such large amounts of such copper compounds generally accelerate corrosion of sensitive bearing metals. Also, while many compounds appear to have very desirable properties when subjected to some laboratory tests, they do not exhibit such properties when tested in an engine, particularly under conditions of heavy-duty service.

It is an object of this invention to provide new, improved and more stable lubricants. Another object is to provide lubricating oils for internal combustion engines and particularly for heavy-duty service. A further object is to provide more stable lubricants which can be employed in internal combustion engines over longer periods of time with the formation of less deposits on the engine and with less corrosion of sensitive bearing metals. A still further object is to provide a lubricant which is more satisfactory in internal combustion engines under heavy-duty service. Other objects are to provide new compositions of matter and to advance the art.

The above and other objects of our invention may be accomplished by dissolving in a petroleum lubricating oil, from 50 to about 1000 parts of copper per one million parts of oil, here-

inafter abbreviated P. P. M., in the form of oil-soluble non-ionogenic organic compounds of copper in the presence of a small proportion, sufficient to impart substantial oil-stabilizing properties to the copper, of sulfur in the form of oil-soluble organic sulfur compounds. We have found that when such copper and sulfur compounds are employed in accordance with our invention, the deterioration of the lubricating oil is largely inhibited and lubricating oils of greatly improved properties are obtained. This is particularly apparent when such lubricating oils are employed in internal combustion engines under heavy-duty service, wherein the copper and the sulfur cooperate to stabilize the oil against deterioration so that the engines can be operated with such lubricating oils over long periods of time without causing objectionable increase in the viscosity of the oils, objectionable corosions of sensitive bearing metals and the formation of objectionable amounts of deposits on the parts of the engines.

By an oil soluble non-ionogenic copper compound we mean a copper compound soluble to the extent of at least 50 P. P. M. copper in a lubricating oil and having substantially no tendency to liberate copper ions. Whether or not an organic copper compound is ionogenic may readily be determined by observing whether or not copper is extracted by an aqueous solution of a weak acid from a solution of the copper compound in a hydrocarbon solvent. For example, the following procedure is a satisfactory and convenient qualitative method for determining whether or not an organic copper compound is ionogenic. An approximately 1% solution of the copper compound in benzene is shaken vigorously for one minute at room temperature with an equal volume of a 10% aqueous solution of tartaric or citric acid. The mixture is then allowed to separate into an upper benzene layer and a lower aqueous layer. If the copper compound is ionogenic, it will be found that the copper has been removed from the benzene solution. This will be shown by a disappearance of the color of the copper compound from the benzene layer. It will also be shown by the presence of copper in the aqueous layer, the copper imparting a pale blue color to the aqueous solution. On addition of excess ammonium hydroxide to a sample of the aqueous layer, the characteristic deep blue color of cuprammonium ions appears. This test is quite sensitive, as little as 50 P. P. M. ionogenic copper in the original benzene solution being sufficient to impart a perceptible blue color on addition of excess ammonium hydroxide to a sample of the aqueous layer. If the copper compound is non-ionogenic, it will be found that substantially no copper has been removed from the benzene solution. The benzene layer will retain the characteristic color of the copper compound and the aqueous layer will not turn blue on addition of excess ammonium hydroxide.

Certain precautions must be observed in applying the above test. The test is so sensitive that copper will be found in the aqueous layer when testing non-ionogenic copper compounds containing, as impurities, small amounts of ionogenic copper compounds. In the case of a few ionogenic copper compounds, a green color will be obtained instead of blue on adding excess ammonium hydroxide to the aqueous layer. If the qualitative test appears to be in any way abnormal or difficult to interpret, it should be confirmed by a quantitative test. This is accom-

plished by analyzing the benzene solution of the copper compound for total copper by quantitative methods both before and after the above-described extraction. If the copper compound is ionogenic, it will be found that the benzene solution contains substantially no copper after extraction. If the copper compound is non-ionogenic, it will be found that the benzene solution, after extraction, contains substantially as much copper as before extraction. When a mixture of ionogenic and non-ionogenic copper compounds is tested, the amount of copper, remaining in the benzene solution after extraction, represents the amount of non-ionogenic copper in the mixture, and the amount of copper, removed by extraction, represents the amount of ionogenic copper in the mixture.

It will be obvious to those skilled in the art of analytical chemistry that, with suitable modifications, this quantitative test is capable of a variety of applications. For example, extraction of a lubricating oil, containing copper compounds, with excess aqueous tartaric or citric acid will separate ionogenic (extracted) and non-ionogenic (not extracted) copper, and the amount of each present in the oil can be quantitatively determined. If the lubricating oil is viscous it may be necessary to prolong the time of extraction or to employ a light hydrocarbon, such as benzene or solvent naphtha, as a thinner in order to obtain quantitative extraction of the ionogenic copper. It should be noted that we employ a weak acid, preferably tartaric acid or citric acid, in the above tests and conduct our extractions at room temperature, 20-30° C. Strong acids, such as hydrochloric acid or sulfuric acid, will extract ionogenic copper but also tend to destroy the non-ionogenic copper compounds. Higher temperatures may be employed for the extraction, but these more severe conditions should not be used because they may give false results due to breaking down or altering the copper-containing molecules.

In our co-pending application Serial No. 440-202, filed April 23, 1942, we have disclosed the stabilization of lubricating oils by incorporating therein from 50 to about 500 P. P. M. of copper together with from about 0.1% to about 0.5% of sulfur. In such application we have disclosed oil soluble compounds of copper generally, including ionogenic as well as non-ionogenic compounds of copper and claim such class broadly and certain ionogenic compounds specifically.

It has been found that the non-ionogenic copper compounds are superior to the ionogenic copper compounds as stabilizers for the lubricating oils and inhibiting corrosion of sensitive bearing metals. When the ionogenic compounds are employed, corrosion of sensitive bearing metals increases rapidly as the amount of copper in the oil is increased above 500 P. P. M., and when amounts substantially above 500 P. P. M. are employed, frequently accelerate rather than inhibit such corrosion. On the other hand, non-ionogenic copper compounds may be employed in such amounts as to produce concentrations of copper as high as 1000 P. P. M., and in some cases as high as 2000 P. P. M. or more and still materially inhibit corrosion of sensitive bearing metals by the oils.

Ionogenic copper compounds include copper derivatives of carboxylic acids, ketonates, phenates, and the purely inorganic salts of copper such as the sulphates, nitrates and halides. Complexes of these copper derivatives, with organic compounds, remain ionogenic. Some of the cop-

per derivatives are quite effective in improving oil condition and engine cleanliness. However, they tend to increase rather than retard bearing corrosion, unless their concentration in the oil is carefully controlled within quite narrow limits. Other ionogenic copper compounds are, in general, only moderately effective in improving oil condition and engine cleanliness and retarding bearing corrosion. The non-ionogenic compounds on the other hand, are not only effective to retard bearing corrosion in a wider range of copper but are also more effective in general in improving oil condition and engine cleanliness and in retarding bearing corrosion. Furthermore, the non-ionogenic copper compounds are more resistant to extraction from the oils by acids and alkalies during the processing and storage of the lubricating oils containing them.

The non-ionogenic copper compounds of our invention may be added to the oils in such proportion as to provide concentrations of copper as low as 50 P. P. M. and in some cases as high as 2000 P. P. M. or more. When employed in such proportions, the stability of the oils will be improved. In general, we prefer not to employ the copper compounds in proportions such as to provide copper in concentrations substantially above 1000 P. P. M., since the optimum results are obtained with concentrations below 1000 P. P. M. of copper and hence no additional benefit is obtained by employing concentration materially above 1000 P. P. M. Accordingly, the addition of more than 1000 P. P. M. of copper is wasteful and uneconomical. When the copper compound is employed in such proportion as to provide from 50 to about 200 P. P. M. of copper, it is generally essential to have present in the oil, at least 0.1% of sulfur in the form of oil-soluble sulfur compounds. When the concentration of copper is increased above 200 P. P. M., such amount of sulfur is not necessary and when the proportion of copper approaches 500 P. P. M. and above, no sulfur may be necessary. However, it will usually be desired to have present in the oil, from about 0.1% to about 0.5% of sulfur, since such sulfur is effective to materially increase the stabilizing effect of the copper. Usually the optimum results will be obtained when the concentration of copper in the oil is within the range of about 100 to about 500 P. P. M., and we preferably employ the copper compounds in such range. However, it should be noted that all oil-soluble copper compounds are not equally effective on a copper basis. The optimum concentration depends upon the nature of the copper compound, the nature of the lubricating oil employed, and the degree of stabilization desired and must be determined experimentally for each compound and each oil.

Some of the more important classes of non-ionogenic copper compounds are copper mercaptides, copper dialkyl dithiocarbamates and copper trithiocarbonates. Representative members of these classes, which have proved to be particularly desirable, are:

Cuprous pentadecyl-8 mercaptide

Cuprous cetyl mercaptide

Copper-treated sulfurized dehydrated "Ocenol"

Cupric dibutyl dithiocarbamate

Cupric diethyl dithiocarbamate

Cuprous trithiocarbonate from pinene

Cuprous pentadecyl-8 trithiocarbonate

Cuprous octyl trithiocarbonate

The preferred class of non-ionogenic copper

compounds is the class of oil-soluble copper mercaptides and particularly the oil-soluble copper mercaptides of aliphatic mercaptans. Of these, we particularly prefer the copper mercaptides of the long chain aliphatic mercaptans. Particularly desirable oil-soluble copper mercaptides are those derived from petroleum and petroleum products. Such mercaptides are comparatively cheap and readily available. The methods of making mercaptans from petroleum products are well known in the art and include, among others, reacting halogenated petroleum fractions with sodium hydrosulfite, and reacting olefins, derived from petroleum, with hydrogen sulfide. The mercaptans, naturally present in petroleum fractions or produced therein during refining processes, may also be isolated and employed for the preparation of copper mercaptides. Mercaptans from petroleum fractions are usually obtained as mixtures of mercaptans of varying chain lengths and structures. In the case of mixtures which contain mercaptans that give insoluble copper salts, such mercaptans may be removed from the mixture by fractional distillation or by other methods prior to the preparation of copper mercaptides or, if desired, copper mercaptides may be prepared from the crude mixture and the oil-soluble copper mercaptides may then be isolated by dissolving them from the mixture into a lubricating oil or other hydrocarbon solvent. The mercaptans may be converted to copper mercaptides by treatment with a copper salt, such as cupric sulfate or cupric acetate, but it is preferable to employ a cuprous salt, such as ammoniacal cuprous chloride, because better yields of mercaptides will be obtained thereby. Crude mixtures of oil-soluble copper mercaptides, derived from petroleum fractions and containing, as by-products or impurities, sulfur compounds such as organic sulfides, disulfides and the like, are suitable for addition to lubricating oils in accordance with our invention. Also, if desired, pure copper mercaptides, such as cuprous cetyl mercaptide, isolated from crude mixtures or made from pure hydrocarbons, such as cetene, obtained from petroleum, may be employed.

Particularly desirable compounds are the copper-treated sulfurized unsaturated compounds. The copper-treated sulfurized unsaturated compounds are the products obtained by sulfurizing an unsaturated compound, generally by treating it with sulfur with or without a catalyst at temperatures from about 130° C. to about 200° C., and then treating such sulfurized product with metallic copper or a copper salt. The preferred sulfurized unsaturated compounds, which are to be employed to produce the copper treated compounds, are the sulfurized unsaturated dehydrated alcohols prepared as disclosed in the co-pending application of F. B. Downing and R. G. Clarkson, Serial No. 440,201 filed April 23, 1942. The process, described in more detail in such application, comprises dehydrating unsaturated long chain alcohols in the presence of catalysts, such as fuller's earth at temperatures of from about 200° C. to about 300° C., whereby the alcohols are largely converted to unsaturated ethers. The resulting dehydrated products are then sulfurized by treatment with sulfur in the presence of a catalyst at temperatures of from about 130° C. to about 200° C. By "long chain," we mean compounds containing a carbon chain of at least 10 carbon atoms. The preferred compounds are the sulfurized dehydrated unsaturated "Ocenols." The term "Ocenols" is generally employed by

those skilled in the art to designate the mixture of unsaturated long chain alcohols obtained by the hydrolytic reduction of unsaturated natural oils from vegetable, fish and animal sources, representative oils being sperm oil, beef tallow, lard oil, cottonseed oil, olive oil, corn oil, rapeseed oil, menhaden oil, soyabean oil, linseed oil and China-wood oil.

The copper treatment of a sulfurized unsaturated compound has the dual advantage of introducing copper into the compound and of removing any unreacted or loosely-bound sulfur that may be present. The copper treatment may be accomplished at temperatures as low as 60° C. or as high as 200° C., but temperatures of about 100° C. will usually be preferred. It is usually sufficient to stir the sulfurized compound with powdered copper or a copper salt at a temperature of about 100° C. The amount of copper employed and the time and temperature of heating will depend on the amount of copper desired in the product and the nature of the sulfurized unsaturated compound. It is preferable to add the copper or copper salt slowly in small portions rather than in one batch. When the sulfurized unsaturated compound contains appreciable quantities of unreacted or loosely bound sulfur, the first portions of copper added react with this sulfur and remove it, presumably as copper sulfide, and only a little copper is introduced into the sulfurized unsaturated compound. When all the unreacted or loosely bound sulfur has been removed, further additions of copper rapidly increase the copper content of the sulfurized unsaturated compound. Copper compounds, that may be employed instead of copper powder, include cuprous chloride, cupric acetate, cupric oxide and cuprous cyanide. When the desired amount of copper has been introduced into the sulfurized unsaturated compound, the mixture is filtered or centrifuged from any copper sulfide or unreacted copper and is then ready for use as an additive for lubricating oils.

We do not know the exact structure of the oil-soluble copper compounds, obtained by treating sulfurized unsaturated compounds with copper or a copper salt. Oil-soluble compositions containing about 0.25-3.0% copper and about 6-20% sulfur are easily obtainable by this method and such compositions are high effective when employed in accordance with our invention.

Another preferred class of non-ionogenic copper compounds comprises the copper dialkyl dithiocarbamates. The members of this class, in which the alkyl groups contain a total of six or more carbon atoms, are oil-soluble. The oil-soluble cupric dialkyl dithiocarbamate are excellent stabilizers for lubricating oils.

The oil, to be employed as the lubricant, may be any of the usual mineral oils, such as the petroleum lubricating oils ordinarily employed in the lubrication of internal combustion engines. It is not essential that the lubricating oil be highly refined, as partially refined and mildly refined oils will respond to the treatment of our invention.

Oil-soluble sulfur compounds, that may be used in conjunction with copper compounds in accordance with our invention, include mercaptans, sulfides, disulfides, polysulfides, thioethers, thiophenols, thiocarbamates, xanthates, thio acids, dithio acids, sulphones, thioamides, and mixtures thereof. Specific examples of some of these types include dibenzyl disulfide, dipinane

disulfide, dicyclohexyl disulfide, dibenzyl sulfide, dioctyl sulfide, dibutyl sulfone, pinane mercaptan, pentadecane-thiol-8, triphenyl phosphine sulfide, 1,2-bis (benzylthio) ethane, dithiobis-diamyl formate, and dithiobis (dibutyl thio formamide). Most lubricating oils contain an appreciable quantity of dissolved naturally occurring sulfur compounds. We have found that these naturally occurring sulfur compounds are also effective when used in conjunction with copper compounds in accordance with our invention. Accordingly, we include the natural sulfur content in the oil when speaking of our preferred concentrations of sulfur. By an oil-soluble sulfur compound, we mean a compound that is sufficiently soluble in a lubricating oil to give a permanent solution at ordinary temperatures containing at least 0.10% sulfur. It should be noted that sulfur compounds behave differently from elemental sulfur. The former enhance the stabilizing action of copper compounds, while the latter detracts from such stabilizing action. Accordingly, we specifically exclude elemental sulfur as a sulfur compound.

The products, obtained by sulfurizing unsaturated compounds, are particularly useful oil-soluble sulfur compounds, when employed in accordance with our invention. It will be understood that an unsaturated compound is an organic compound which contains one or more olefinic double bonds. These compounds include the sulfurized natural oils from vegetable, fish, and animal sources, as well as sulfurized synthetic unsaturated compounds. Sulfurized sperm, lard, corn and menhaden oils and sulfurized terpenes may be mentioned as examples of sulfurized natural oils. Examples of sulfurized synthetic unsaturated compounds include the products obtained by sulfurizing cetene, abietene, cyclohexene, dihydronaphthalene, menthene, dipentene, terpinene, terpinolene, oleyl alcohol, abietyl alcohol, methyl oleate and methyl abietate. Mixtures of sulfurized unsaturated compounds are equally suitable. The exact chemical structure of these sulfurized unsaturated compounds is not definitely known. It is known, however, that each double bond of such an unsaturated compound will ordinarily react with one, two, or three atoms of sulfur. We prefer to employ compounds which contain not more than one atom of sulfur for each double bond present. Sulfur, in excess of this quantity, tends to function as elemental sulfur in detracting from the stabilizing action of copper compounds and hence is undesirable.

The preferred sulfurized unsaturated compounds to be employed in combination with the copper compounds, in accordance with our invention, are sulfurized unsaturated dehydrated alcohols, prepared as described in the co-pending application of F. B. Downing and R. G. Clarkson, Serial No. 440,201 filed April 23, 1942.

It has been found that when lubricating oils are employed in internal combustion engines, the properties of the lubricating oils are materially affected by the character of the fuel employed in the engine. It has been found that, when the motor fuel employed in an internal combustion engine contains tetra-ethyl lead, deterioration of the lubricating oil and corrosion of sensitive bearing metals are materially increased. On the other hand, it has been found that, when the lubricating oils of our invention are employed in internal combustion engines operating on motor oils containing tetra-ethyl lead, the effec-

tiveness of the copper compounds in stabilizing the lubricating oils, is very materially increased. Also, our compounds are still very effective to inhibit corrosion of sensitive bearing metals even when the motor fuel contains substantial amounts of tetra-ethyl lead. The use of motor fuels, containing tetra-ethyl lead, in combination with the lubricants of our invention is disclosed more specifically and is claimed in the co-pending application of J. H. Fuller and J. R. Sabina, Serial No. 440,250 filed April 23, 1942, for "Method of operating internal combustion engines."

The most satisfactory method of determining the stability of a lubricant in an internal combustion engine is by actual use of the lubricant in the engine. We employ the following engine test, which correlates well with results obtained in the field. Six-cylinder 1940 and 1941 model Chevrolet engines (in some cases fitted with one copper-lead bearing) are operated on a block mounting at a speed of 3150 R. P. M. (equivalent to a road speed of 60 miles per hour) against a load of 35 brake horse-power (equivalent to that obtained in road operation) applied by means of a dynamometer. The oil in the sump is maintained at 280° F. and the cooling jacket liquid at 200° F. The test is run for 66½ hours (corresponding to road operation for 4000 miles), except in cases where the oil deterioration is so extensive that such lengthy operation is impractical. The degree of deterioration of the oil in this test corresponds directly to that obtained in equal periods of heavy-duty service and is indicative of that observed in longer periods of less severe service.

The following ratings are employed to determine the stability of the oil and its effect on the engine. Samples of the oil used are removed from the crankcase at intervals and analyzed for total sludge (naphtha insolubles) and asphaltenes (chloroform solubles) by the method described in J. Ind. Eng. Chem., Anal. Ed. 6, 419 (1934) and for viscosity rise and neutralization number by the well-known A. S. T. M. methods. On the basis of these analyses, the condition of the oils is rated as excellent, good, fair, poor or bad. At the end of the run, the engine is disassembled, inspected and rated as to cleanliness. In the system of cleanliness rating employed, a clean engine would

5  
10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955  
8960  
8965  
8970  
8975  
8980  
8985  
8990  
8995  
9000  
9005  
9010  
9015  
9020  
9025  
9030  
9035  
9040  
9045  
9050  
9055  
9060  
9065<br

The mixture was then cooled to 200° C. and sulfurized by stirring with 15 parts of sulfur for 3 hours at 195-205° C. This product is representative of the sulfurized unsaturated compounds disclosed and claimed in the co-pending application of F. B. Downing and R. G. Clarkson, hereinbefore referred to. The product, thus obtained, was then copper treated. This was accomplished by slowly adding 16 parts of copper powder with stirring during 10 hours at 100-110° C. The mixture was then filtered from fuller's earth, copper sulfide and unreacted copper powder. The filtrate was copper-treated sulfurized dehydrated "Ocenol" as a dark-red oil containing 7.43% S and 0.63 Cu. This material is designated I. Two other samples of copper-treated sulfurized dehydrated "Ocenol," prepared in a similar manner, are designated II and III. II contained 8.77% S and 1.19% Cu, and III contained 8.89% S and 2.15% Cu. These materials were tested in Chevrolet engines, as previously described, and the results of the tests are given in Table II.

tion primarily, if not entirely, through protection of the oil from the deleterious effects of oxidation during use in the engine. The concentrations employed are insufficient to produce any worthwhile detergency or lubricity in the oil, and the non-ionogenic copper compounds appear to function as antioxidants rather than as detergents or film strength improvers. Furthermore, the lubricating oil compositions disclosed are free-flowing liquid lubricants suitable for crankcase use and are not greases.

While we have disclosed the preferred embodiments of our invention, it will be understood that such specific embodiments are given for illustrative purposes only and that various modifications may be made therein without departing from the spirit or scope of our invention. For example, we have disclosed generally, the use of single copper compounds. It will be apparent that mixtures of any two or more oil-soluble non-ionogenic copper compounds of our invention may be employed, if desired. Accordingly, we intend

TABLE II  
*Effect of copper-treated sulfurized dehydrated "Ocenol" on oil condition, engine cleanliness and bearing corrosion.*

| Oil | Additive  | P. P. M.<br>Cu in<br>oil | Total<br>percent<br>S in oil | Hours<br>tested | Oil con-<br>dition<br>rating | Engine<br>cleanli-<br>ness<br>rating | Cu-Pb<br>corro-<br>sion |
|-----|-----------|--------------------------|------------------------------|-----------------|------------------------------|--------------------------------------|-------------------------|
| A   | None      | 0                        | 0.23                         | 66%             | Bad                          | 56.5                                 | 1.05                    |
| A   | 2.08% I   | 129                      | 0.38                         | 66%             | Excellent                    | 94.0                                 | 0.59                    |
| B   | None      | 0                        | 0.06                         | 33%             | Bad                          | 63.0                                 | 1.20                    |
| B   | 2.08% I   | 129                      | 0.21                         | 66%             | Excellent                    | 94.5                                 | 0.08                    |
| C   | None      | 0                        | 0.26                         | 33%             | Bad                          | 60.5                                 | 0.03                    |
| C   | 2.08% I   | 129                      | 0.41                         | 66%             | Good                         | 86.0                                 | 0.11                    |
| D   | None      | 0                        | 0.31                         | 33%             | Bad                          | 53.0                                 | (1)                     |
| D   | 1.71% II  | 203                      | 0.46                         | 66%             | Good                         | 85.5                                 | (1)                     |
| E   | None      | 0                        | 0.16                         | 50              | Bad                          | 42.0                                 | 0.85                    |
| E   | 0.75% III | 164                      | 0.23                         | 66%             | Good                         | 82.0                                 | 0.95                    |
| F   | None      | 0                        | 0.11                         | 66%             | Bad                          | 66.0                                 | 1.90                    |
| F   | 2.08% I   | 129                      | 0.26                         | 66%             | Good                         | 83.0                                 | 0.10                    |

<sup>1</sup> Oil D was non-corrosive.

The tests, the results of which are shown in Table II above, were conducted with the engines operating on gasoline having incorporated therein 1 cc. per gallon of tetra ethyl lead as a well known standard commercial composition which also contained alkyl halides.

While the stabilizing action of non-ionogenic copper compounds on lubricants for internal combustion engines is most striking in so-called heavy-duty service, a similar effect is also obtained in less severe service. Internal combustion engines in which these additives may be employed with beneficial results include engines designed for use in passenger automobiles, trucks, tanks, buses, tractors, aircraft and stationary and semi-stationary power plants. Furthermore, the beneficial action of these additives is not limited to any particular type or kind of oil. Excellent results can be obtained in mildly refined as well as in highly refined oils and in paraffinic base oils as well as in naphthenic and asphaltic base oils. The non-ionogenic copper compounds may also be employed in conjunction with other additives such as pour point depressants, viscosity index improvers, thickeners, detergents and the like.

We do not know the exact mechanism by which the non-ionogenic copper compounds function as lubricant stabilizers. They appear to func-

to cover our invention broadly as in the appended claims.

We claim:

1. A lubricant comprising a petroleum lubricating oil having dissolved therein from 50 to 1000 P. P. M. of copper in the form of an oil-soluble non-ionogenic organic compound of copper and a small proportion, sufficient to impart substantial oil-stabilizing properties to the copper, of sulfur in the form of oil-soluble organic sulfur compounds.
2. A lubricant comprising a petroleum lubricating oil having dissolved therein from 50 to 1000 P. P. M. of copper in the form of an oil-soluble non-ionogenic organic compound of copper and from about 0.1% to about 0.5% of sulfur in the form of oil-soluble organic sulfur compounds.
3. A lubricant comprising a petroleum lubricating oil having dissolved therein from 50 to 1000 P. P. M. of copper in the form of an oil-soluble non-ionogenic organic compound of copper and from about 0.1% to about 0.5% of sulfur in the form of oil-soluble organic sulfur compounds, at least a substantial proportion of which are sulfurized unsaturated organic compounds containing a maximum of one sulfur atom for each effective double bond.
4. A lubricant comprising a petroleum lubricating oil having dissolved therein from 50 to 1000

P. P. M. of copper in the form of an oil-soluble non-ionogenic organic compound of copper and from about 0.1% to about 0.5% of sulfur in the form of oil-soluble organic sulfur compounds, at least a substantial part of which are sulfurized unsaturated ethers containing a maximum of one sulfur atom for each effective double bond.

5. A lubricant comprising a petroleum lubricating oil having dissolved therein from 50 to 1000 P. P. M. of copper in the form of an oil-soluble non-ionogenic organic compound of copper and from about 0.1% to about 0.5% of sulfur in the form of oil-soluble organic sulfur compounds, at least a substantial proportion of which are sulfurized unsaturated dehydrated alcohols obtained by the reduction of an unsaturated natural oil which sulfurized dehydrated alcohols contain a maximum of one sulfur atom for each effective double bond.

6. A lubricant comprising a petroleum lubricating oil having dissolved therein from 50 to 1000 P. P. M. of copper in the form of an oil-soluble copper mercaptide and a small proportion, sufficient to impart substantial oil-stabilizing properties to the copper, of sulfur in the form of oil-soluble organic sulfur compounds.

7. A lubricant comprising a petroleum lubricating oil having dissolved therein from 50 to 1000 P. P. M. of copper in the form of an oil-soluble copper mercaptide of an aliphatic mercaptan and a small proportion, sufficient to impart substantial oil-stabilizing properties to the copper, of sulfur in the form of oil-soluble organic sulfur compounds.

8. A lubricant comprising a petroleum lubricating oil having dissolved therein from 50 to 1000 P. P. M. of copper in the form of an oil-soluble copper mercaptide of a long-chain aliphatic mercaptan and a small proportion, sufficient to impart substantial oil-stabilizing properties to the copper, of sulfur in the form of oil-soluble organic sulfur compounds.

9. A lubricant comprising a petroleum lubricating oil, normally containing substantially less than 0.5% sulfur, and having dissolved therein a non-ionogenic copper-treated sulfurized unsaturated organic compound wherein both the copper and the sulfur are chemically combined, there being a maximum of one sulfur atom for each double bond in the compound, the organic compound being dissolved in such proportion that the oil contains from 50 to about 500 P. P. M. of copper and from about 0.1% to about 0.5% sulfur.

10. A lubricant comprising a petroleum lubricating oil, normally containing substantially less than 0.5% sulfur, and having dissolved therein a non-ionogenic organic compound containing chemically combined copper and sulfur, which organic compound is a copper-treated sulfurized dehydrated mixture of unsaturated long chain alcohols, the organic compound being dissolved in the lubricating oil in such proportion that the oil contains from 50 to 500 P. P. M. of copper and from about 0.1% to about 0.5% sulfur.

11. A lubricant comprising a petroleum lubricating oil, normally containing substantially less than 0.5% sulfur, and having dissolved therein a non-ionogenic organic compound containing chemically combined copper and sulfur, which

organic compound is a copper-treated sulfurized dehydrated mixture of unsaturated long chain alcohols derived from an unsaturated fatty oil, the organic compound being dissolved in the lubricating oil in such proportion that the oil contains from 50 to 500 P. P. M. of copper and from about 0.1% to about 0.5% sulfur.

12. A lubricant comprising a petroleum lubricating oil, normally containing substantially less than 0.5% sulfur, and having dissolved therein a non-ionogenic organic compound containing chemically combined copper and sulfur, which organic compound is a copper-treated sulfurized dehydrated mixture of unsaturated long chain alcohols derived from sperm oil, the organic compound being dissolved in the lubricating oil in such proportion that the oil contains from 50 to 500 P. P. M. of copper and from about 0.1% to about 0.5% sulfur.

13. A lubricant comprising a petroleum lubricating oil having dissolved therein from 50 to 1000 P. P. M. of copper in the form of an oil-soluble dialkyl dithiocarbamate of copper and a small proportion, sufficient to impart substantial oil-stabilizing properties to the copper, of sulfur in the form of oil-soluble organic sulfur compounds.

14. A lubricant comprising a petroleum lubricating oil having dissolved therein from 50 to 1000 P. P. M. of copper in the form of an oil-soluble dialkyl dithiocarbamate of copper in which the alkyl groups contain a total of at least six carbon atoms and from about 0.1% to about 0.5% of sulfur in the form of oil-soluble organic sulfur compounds.

15. A lubricant comprising a petroleum lubricating oil having dissolved therein from 50 to 1000 P. P. M. of copper in the form of cupric dibutyl dithiocarbamate and from about 0.1% to about 0.5% of sulfur in the form of oil-soluble organic sulfur compounds.

16. A heavy-duty internal combustion engine lubricant comprising a petroleum lubricating oil having dissolved therein from 50 to 1000 P. P. M. of copper in the form of an oil-soluble non-ionogenic organic compound of copper and a small proportion, sufficient to impart substantial oil-stabilizing properties to the copper, of sulfur in the form of oil-soluble organic sulfur compounds.

17. A heavy-duty internal combustion engine lubricant comprising a petroleum lubricating oil, normally containing substantially less than 0.5% sulfur, and having dissolved therein a non-ionogenic copper-treated sulfurized unsaturated organic compound wherein both the copper and the sulfur are chemically combined, there being a maximum of one sulfur atom for each double bond in the compound, the organic compound being dissolved in such proportion that the oil contains from 50 to about 500 P. P. M. of copper and from about 0.1% to about 0.5% sulfur.

18. A lubricant comprising a petroleum lubricating oil having dissolved therein from 50 to 1000 P. P. M. of copper in the form of cuprous pentadecyl-8 mercaptide and from about 0.1% to about 0.5% of sulfur in the form of oil-soluble organic sulfur compounds.

FREDERICK B. DOWNING,  
HOWARD M. FITCH.